

[54] METHOD AND COMPOSITION OF MIXED  
BASO<sub>4</sub> AND SRSO<sub>4</sub> FOR POLISHING A  
PHOTOCONDUCTOR SURFACE

[75] Inventors: **Kazunori Matsuo**, Tokyo; **Kohji Suzuki**; **Katutsohi Endo**, both of Yokohama, all of Japan

[73] Assignee: **Ricoh Co., Ltd.**, Tokyo, Japan

[22] Filed: **Jan. 24, 1973**

[21] Appl. No.: **326,561**

[30] Foreign Application Priority Data

Feb. 17, 1972 Japan ..... 47-16724

[52] U.S. Cl. ..... 252/164; 252/89; 252/163

[51] Int. Cl. ..... C09g 1/02; C11d 7/50

[58] Field of Search ..... 252/89, 163, 164; 51/307

[56] References Cited

UNITED STATES PATENTS

|           |         |                |               |
|-----------|---------|----------------|---------------|
| 2,503,744 | 4/1950  | Kenney et al.  | ..... 252/89  |
| 2,739,129 | 3/1956  | Manchot        | ..... 252/89  |
| 3,702,303 | 11/1972 | Clemens et al. | ..... 252/163 |

FOREIGN PATENTS OR APPLICATIONS

937,122 9/1963 United Kingdom ..... 252/163

OTHER PUBLICATIONS

Gmelins Handbuch der Anorganischen Chemie, 8th Ed., Barium, System No. 30, p. 388, Verlag Chemie, G.m.b.H.(1932) Berlin. QD 151 G5.

Gmelins Handbuch der Anorganischen Chemie, 8th Ed. Suppl., Barium, System No. 30, pp. 533-534, Verlag Chemie, GmbH (1960) Weinheim/Bergstrasse. QD 151 G5.

Primary Examiner—Benjamin R. Padgett

Assistant Examiner—E. A. Miller

Attorney, Agent, or Firm—Cooper, Dunham, Clark, Griffin & Moran

[57] ABSTRACT

Method for polishing the surface of a photoconductor consisting essentially of amorphous selenium to recover the surface properties of the photoconductor to the original level which has deteriorated by repeated use or aging, and polishing material for such use.

5 Claims, No Drawings

**METHOD AND COMPOSITION OF MIXED BASO<sub>4</sub>  
AND SRSO<sub>4</sub> FOR POLISHING A  
PHOTOCOCONDUCTOR SURFACE**

**BACKGROUND OF THE INVENTION**

In the xerographic process, amorphous selenium is preferably used as a photoconductor. A layer of amorphous selenium constitutes a photoconductive layer for xerographic plates. The layer of amorphous selenium is formed on a conductive substrate such as a copper or aluminium plate by vacuum evaporation. The xerographic process consists of the steps of:

1. Charging a surface of photoconductive layer by a corona discharge,
2. forming an electrostatic latent image on the photoconductive layer by image-wise exposure to light,
3. electrically precipitating toners (in powder form) on the latent image to form visible image,
4. transferring the visible toner image to a transfer medium such as a paper sheet, and
5. affixing the transferred toner image to the paper sheet by fusing.

The toners are powders generally made of a mixture of carbon black and synthetic resin such as a styrene-butadiene copolymer. Accordingly, the synthetic resin is melted by fusing to affix the toners to the paper sheet. All of this is well known to those skilled in the art. A D.C. voltage of 6kV (or 5kV) is applied in the corona discharge and generally, an acceptance potential of about 750V (or about 700V) is obtained. The acceptance potential which may be obtained is reduced to the extent of about 660V (or 600V) by repeatedly using the photoconductive layer, for example, 10 thousands times. This reduction of the acceptance potential is caused by the following factors:

1. the attachment of toners or dust (in the air) to the surface of the photoconductor,
2. the roughness of the surface of the layer resulting from the attachment of the dust, and
3. the change in quality of the surface attributed to aging.

Accordingly, in order to recover the deteriorated photoconductor to obtain the original acceptance potential, it is required to clean or polish the surface of the photoconductor. For this purpose, various polishing (or cleaning) materials or methods have been proposed. For instance, there are disclosed cubic salts e.g. NaCl or NH<sub>4</sub>Cl in U.S. Pat. No. 2,484,782, BaSO<sub>4</sub> metaphosphate salts in U.S. Pat. No. 2,772,991, and kieselguhr and etherified cellulose in U.S. Pat. No. 3,100,726. Further, it is well known to those skilled in the art that a dispersion of Ce<sub>2</sub>O<sub>3</sub> in hydrocarbon is useful as a polishing material.

The use of solvents by which a toner film formed on the surface of the photoconductor is removed is also known. One such solvent is isopropyl alcohol.

However, these procedures to polish or clean the surface of the photoconductor have not been completely satisfactory.

It is an object of the present invention to provide an improved polishing material and method for use in polishing a surface of amorphous selenium photoconductors.

**SUMMARY OF THE INVENTION**

The present invention relates to polishing materials and methods for polishing the surface of amorphous selenium photoconductors.

As previously stated, the surface of photoconductive amorphous selenium, which is used in the xerographic process, will deteriorate in quality by repetitive use. It has been found that:

1. in order to recover the deteriorated surface, it is effective and efficient to polish the surface with strontium sulfate (SrSO<sub>4</sub>) or barium sulfate (BaSO<sub>4</sub>) powders, or preferably a mixture thereof, and
2. it is most effective and efficient to polish the surface with absorbent cotton (or cotton wool) holding a suspension of a mixture of SrSO<sub>4</sub> and BaSO<sub>4</sub> in an organic solvent such as isopropyl alcohol.

Photoconductive layers used in this invention may be prepared as follows: the photoconductive layer i.e. an amorphous selenium layer is formed on a conductive support (for example, an aluminum drum having a diameter of 17cm) by depositing a thin layer (about 50 $\mu$  thick) of selenium by vacuum evaporation. The dark resistivity of a selenium layer thus formed is 10<sup>14</sup> $\Omega$ .cm.

Toners used in this invention may be made as follows: a mixture of one part by weight of carbon black and ten parts by weight of butadiene-styrene copolymer is heated to a temperature of about 200°C. After cooling, the mixture is finely divided to powders having a particle size of from 1 $\mu$  to 20 $\mu$ .

Using the photoconductive layer and the toners as prepared above, xerographic copying process comprising (1) charging by corona discharge of +6kV or +5kV, (2) image-wise exposure to light, (3) development, and (4) transferring was repeated about ten to twenty thousands times.

The deteriorated photoconductive layer thus obtained was polished with absorbent cotton holding each of the polishing materials mentioned below having particle size of 0.1 $\mu$  to 30 $\mu$ . The polishing ability of each of the polishing materials was compared and evaluated, and it was found that strontium sulfate and barium sulfate are most effective.

The polishing materials are as follows: calcium carbonate (CaCO<sub>3</sub>), cerium oxide (Ce<sub>2</sub>O<sub>3</sub>), zirconium oxide (ZrO<sub>2</sub>), magnesium oxide (MgO), titanium oxide (TiO<sub>2</sub>), silicon oxide (SiO<sub>2</sub>), chromium oxide (Cr<sub>2</sub>O<sub>3</sub>), aluminum silicate Al<sub>2</sub>SiO<sub>5</sub>, magnesium silicate (Mg<sub>2</sub>SiO<sub>4</sub>), calcium silicate (Ca<sub>2</sub>SiO<sub>4</sub>), aluminum sulfate (Al<sub>2</sub>(SO<sub>4</sub>)<sub>3</sub>), calcium sulfate (CaSO<sub>4</sub>), strontium sulfate (SrSO<sub>4</sub>), barium sulfate (BaSO<sub>4</sub>), magnesium sulfate (MgSO<sub>4</sub>), zinc sulfide (ZnS), zinc chloride (ZnCl<sub>2</sub>) and kieselguhr.

The above-cited compounds are chemical reagents which are readily available commercially.

SrSO<sub>4</sub> or BaSO<sub>4</sub> solely may be used individually as a polishing materials, but a mixture of SrSO<sub>4</sub> and BaSO<sub>4</sub> in the ratio of 1:5:1 to 1:15 (by weight) is more effective. However, a suspension of said mixture in methyl alcohol, ethyl alcohol, propyl alcohol or isopropyl alcohol is most effective and efficient.

The characteristics of SrSO<sub>4</sub> and BaSO<sub>4</sub> are as shown below:

| Ability of polishing<br>Recover of acceptance<br>potential | SrSO <sub>4</sub><br>high<br>low | ><br>< | BaSO <sub>4</sub><br>low<br>high |
|------------------------------------------------------------|----------------------------------|--------|----------------------------------|
|------------------------------------------------------------|----------------------------------|--------|----------------------------------|

The polishing material of the present invention is used in the manner as illustrated below:

After toners attached to the photoconductive layer have been removed by a light brushing of the layer with soft cotton, the surface is polished by wiping several times with absorbent cotton holding a dispersion of  $\text{SrSO}_4$  or  $\text{BaSO}_4$  in isopropyl alcohol. As the surface is left standing for 20 to 30 seconds after polishing, isopropyl alcohol evaporates and brownish powders remain on the surface. The toner powders can easily be removed by wiping the surface with soft cotton, and then the surface may be wiped with absorbent cotton holding isopropyl alcohol, if desired.

5

10

700-710V by corona discharge of +6kV or +5kV, respectively.

2. After copying process was repeated 15,000 - 20,000 times with toners made of carbon black and butadiene-styrene copolymer, a reduced acceptance potential obtained by corona discharge of +6kV or +5kV was observed.
3. After the surface of the photoconductive layer was respectively polished with polishing materials No. 1 - No. 6, a recovered acceptance potential obtained by corona discharge was measured, and appearance of the surface was observed.

The data and the results are shown in the table below:

15

|                                                      | Polishing material            |        |             |             |        |        |
|------------------------------------------------------|-------------------------------|--------|-------------|-------------|--------|--------|
|                                                      | No. 1                         | No. 2  | No. 3       | No. 4       | No. 5  | No. 6  |
| Corona discharge (kV)                                | 6                             | 6      | 6           | 6           | 5      | 5      |
| Initial acceptance potential (V)                     | 750                           | 760    | 750         | 750         | 700    | 710    |
| Number of repetition of copying process              | 20,000                        | 20,000 | 20,000      | 20,000      | 15,000 | 15,000 |
| Reduced acceptance potential (V)                     | 650                           | 640    | 660         | 660         | 600    | 600    |
| Recovered acceptance potential (after polishing) (V) | 720                           | 750    | 730         | 750         | 670    | 650    |
| Appearance of the surface of photoconductor          | slightly marred and scratched | smooth | very smooth | very smooth | smooth | smooth |

## DESCRIPTION OF THE PREFERRED EMBODIMENTS

The following nonlimiting examples are given by way of illustration only.

### EXAMPLE 1

Polishing materials No. 1 - No. 6 were prepared from the following ingredients:

|       |                                                                                        | Parts by weight |
|-------|----------------------------------------------------------------------------------------|-----------------|
| No. 1 | $\text{SrSO}_4$ (only)                                                                 |                 |
| No. 2 | $\text{BaSO}_4$ (only)                                                                 |                 |
| No. 3 | $\begin{cases} \text{SrSO}_4 \\ \text{BaSO}_4 \end{cases}$                             | 1               |
| No. 4 | $\begin{cases} \text{SrSO}_4 \\ \text{BaSO}_4 \\ \text{Isopropyl alcohol} \end{cases}$ | 10              |
| No. 5 | $\begin{cases} \text{SrSO}_4 \\ \text{BaSO}_4 \end{cases}$                             | 10              |
| No. 6 | $\begin{cases} \text{SrSO}_4 \\ \text{BaSO}_4 \\ \text{Ethyl alcohol} \end{cases}$     | 10              |

Particle sizes of  $\text{SrSO}_4$  and  $\text{BaSO}_4$  were from  $0.1\mu$  to  $30\mu$ .

Tests of the polishing materials No. 1 - No. 6 were carried out in the following way to evaluate their effects:

1. A photoconductive layer consisting of amorphous selenium was prepared, said photoconductive layer having an acceptance potential of 750-760V or

40 As is seen from the above-mentioned data and results, the polishing materials No. 3 - No. 6 made of a mixture of  $\text{SrSO}_4$  and  $\text{BaSO}_4$  are preferred.

### EXAMPLE 2

45 An amorphous selenium photoconductor was allowed to stand for 6 months in the air.

The initial acceptance potential and reduced acceptance potential (after 6 months) obtained were respectively 750V and 650V by corona discharge of 6kV.

50 After the deteriorated surface of photoconductor was polished with polishing materials No. 3, No. 4 and No. 5 of Example 1, a recovered acceptance potential was measured.

The polishing materials No. 3, No. 4 and No. 5 gave respectively recovered acceptance potentials of 740V, 750V and 720V.

55 The polishing material of this invention may also be used in polishing photoconductive surfaces consisting of amorphous selenium containing a small amount of other elements such as tellurium, arsenic, sulfur or thallium.

We claim:

1. Method for polishing a surface of photoconductor consisting essentially of amorphous selenium with polishing material, said polishing material comprising a mixture of strontium sulfate and barium sulfate.

2. Method according to claim 1 wherein said polishing material is a mixture of strontium sulfate and barium sulfate in the ratio of from 15:1 to 1:15 parts by weight.

3. Method according to claim 2 wherein particle sizes of strontium sulfate and barium sulfate are from 0.1  $\mu$  to 30  $\mu$ .

4. Polishing materials for use with photoconductive

amorphous selenium, comprising a mixture of strontium sulfate and barium sulfate in the ratio of from 15:1 to 1:15 parts by weight, the particle size of the strontium sulfate and barium sulfate being from 0.1  $\mu$  to 30  $\mu$ .

5. Polishing material of claim 4 suspended in an alcohol containing from 1 to 3 carbon atoms.

\* \* \* \* \*

10

15

20

25

30

35

40

45

50

55

60

65